

# UNITED STATES PATENT OFFICE.

CHARLES OTTO BOLZ, OF PORT NORFOLK, VIRGINIA.

## ART OF DYEING.

1,321,973.

Specification of Letters Patent. Patented Nov. 18, 1919.

No Drawing.

Application filed November 21, 1917. Serial No. 203,211.

*To all whom it may concern:*

Be it known that I, CHARLES O. BOLZ, a citizen of the United States, residing at Port Norfolk, in the county of Norfolk and State 5 of Virginia, have invented certain new and useful Improvements in the Art of Dyeing, of which the following is a specification:

The present invention relates to the art of dyeing, and more particularly to a 10 method of dyeing cloths, such as wool and silk.

While the method contemplated herein has to do more particularly with the dyeing of cloth a yellow or yellowish coloring, yet 15 in its broader aspect, the invention embraces dyeing in different shades of yellow, as well as different colors, such as tan, and drab by slight changes in the ingredients employed, the duration of treatment, in the 20 various baths, and by interchanging the order of treatment in said baths.

One of the objects of the invention is to provide highly efficient, novel and improved methods of dyeing, which while giving entirely satisfactory results, are of a comparatively inexpensive character, and easy to practice.

Suitable dyes and dyeing processes for coloring in yellow and similar shades, in a 30 manner to withstand wear, light, etc., are in demand at the present time, owing to the scarcity and incident expense of dye materials or ingredients as heretofore largely employed in dyeing operations, and I have 35 discovered a novel and improved method of dyeing materials such as wool and silk, a pleasing coloring having a more brilliant appearance than previously dyed goods, while at the same time preserving the desirable 40 advantages of more expensive methods, more particularly with regard to fixidity and durability of the coloring.

The various advantages and meritorious characteristics of the improved process of 45 dyeing herein contemplated will be appreciated by those skilled in the art to which the invention relates, from the description to follow, but in this connection, as previously noted, it is to be borne in mind that 50 various minor changes may be resorted to, and still be within the spirit of the invention.

In carrying the improved method, it is proposed to subject the cloth or other material 55 to be dyed to the treatment of certain baths whereby to impart to the material

the desirable coloring effect and whereby to render the coloring permanent.

Assuming that it is desirable to color cloths such as wool and silk, yellow, the improved process may be said to reside generally in placing the material to be treated in a bath of hot tannic acid for a desirable interval, maintaining the bath in a hot, and preferably boiling state during this treatment and thereafter, preferably directly, subjecting the goods to a bath of cold lime water, and finally subjecting the goods to a treatment in a bath comprising a weak solution of nitric acid thoroughly mixed 70 with cold water, the nitric acid bath being brought to a boil prior to the introduction of the material, and maintained at a boil during the treatment of the goods therein.

The preferred method may be described 75 in detail as follows:

The tannic acid may be obtained in various ways, but it is preferred in view of the better results accomplished, to employ white oak or water oak for this purpose. 80 After the acid bath has been prepared and brought to a boiling condition the goods are introduced thereinto. Thereupon unslaked lime is placed in a receptacle, and when slaked is allowed to stand for a sufficient interval for the lime water to become clear, when such clear water is drawn off from the lime and placed in a receptacle. After the lime water has arrived at a cool state, the goods are taken from the tannic 90 acid bath, and while still in a warm condition are introduced into the cool lime water. When so introduced the goods are preferably subjected to a stirring action by any suitable means. Thereupon a relatively 95 weak solution of nitric acid is prepared by mixing the same in cold water, and this solution is brought to a boiling condition, when the goods are introduced into the bath thus provided where the goods will remain 100 for the desirable time.

For imparting to the goods a lighter yellow coloring, that intermediate step of the process including the lime water bath may be eliminated, and the goods upon being 105 withdrawn from the tannic acid bath may be introduced directly into the nitric acid solution while in a boiling state.

In order to obtain a tan coloring, the method is somewhat reversed, that is to say 110 the goods to be dyed will first be boiled in a weak solution of nitric acid, and there-

after boiled in the tannic acid bath, and finally subjected to a stirring action in the cold lime water bath.

Should the goods be bleached, it may be 5 desirable, in obtaining the necessary tan coloring to substitute a salt bath for the nitric acid bath.

Now assuming that it is desired to obtain a drab coloring for wool or the like, these 10 goods after being first boiled in the tannic acid solution for the desirable period are removed and directly introduced into the cold lime water bath, while preferably subjected to a stirring operation, and finally the goods 15 are removed and subjected to a bath including a weak solution of blue vitriol dissolved in hot water, which last mentioned bath is brought to a boiling state previous to the introduction of the goods.

20 Though not necessary in all instances, very desirable and satisfactory results are obtained by subjecting the goods previous to any of the above treatments to a preliminary hot salt water bath, since by this treatment 25 the goods are not only thoroughly cleansed prior to the coloring operation, but the pores are partially opened, and fatty materials extracted therefrom, with the result that the cloth is in a most favorable condition to 30 readily receive the coloring material in the subsequent baths.

It has been ascertained that the nitric acid solution, as distinguished from many other acids heretofore employed for similar 35 purposes will render the coloring exceedingly bright and pleasing, and this acid will also open the pores and remove any remaining fat in the fabric thereby allowing the color to more readily stick or adhere to the 40 fabric. It has also been ascertained that goods dyed in the manner above specified will have a permanent and lasting color

largely unaffected by light, water or atmospheric conditions.

What I claim is:

45

1. The art of dyeing which includes subjecting the material to a tannic acid bath, and subsequently to a solution including nitric acid.

2. The improved method of dyeing cloth 50 and the like which consists in boiling the goods in a tannic acid bath, and thereafter subjecting the goods to treatment in lime water and nitric acid solutions.

3. The improved method of dyeing cloth 55 and the like which consists in boiling the goods in a tannic acid solution, removing the goods and introducing the same into a cool lime water bath, and thereafter introducing the goods into a weak solution of nitric acid. 60

4. The improved method of dyeing cloth and the like which consists in boiling the goods in a tannic acid solution, removing the goods, introducing the same into a cool lime water bath, and thereafter introducing the 65 goods into a weak solution of nitric acid, the nitric acid being in a boiling condition.

5. The improved method of dyeing cloth and the like which consists in boiling the goods to be treated in a bath of tannic acid, 70 removing the goods and while hot introducing the same into a cold lime water bath, stirring the goods in the last mentioned bath, removing the goods, and finally subjecting the same to a bath including a solution of 75 nitric acid, the last mentioned bath being in a boiling condition.

In testimony whereof I hereunto affix my signature in the presence of two witnesses.

CHARLES OTTO BOLZ.

Witnesses:

WILLIAM N. SEBRELL,  
OTIS E. BUTLER.